# EUROPEAN PATENT SPECIFICATION

(11) **EP 1 281 777 B1**
(45) Date of publication and mention of the grant of the patent: **23.06.2010**
(21) Application number: 01919779.7
(22) Date of filing: 04.04.2001
(51) Int. Cl.: C21D 8/00, B21B 1/08, C22C 38/00, C22C 38/12

(54) **A METHOD OF PRODUCING A ROLLED H-SHAPED STEEL HAVING UNIFORM MICROSTRUCTURE AND UNIFORM MECHANICAL PROPERTIES**
HERSTELLUNGSVERFAHREN FÜR GEWALZTE H-PROFILSTAHL MIT GLEICHMÄSSIGER MIKROSTRUKTUR UND MECHANISCHENEIGENSCHAFTEN
PROCEDE DE FABRICATION UNE PROFILE EN ACIER LAMINE EN FORME DE H A MICROSTRUCTURE UNIFORME ET PROPRIETES MECANIQUES UNIFORMES

(30) Priority: 04.04.2000 JP 2000102299; 11.04.2000 JP 2000109778; 28.09.2000 JP 2000296547; 05.01.2001 JP 2001000695
(43) Date of publication of application: 05.02.2003
(73) Proprietor: Nippon Steel Corporation, Tokyo 100-8071 (JP)
(72) Inventor: YOSHIDA, Suguru, NIPPON STEEL CORPORATION, Futtsu-shi, Chiba 293-8511 (JP); SATOH, Hironori, C/O NIPPON STEEL CORPORATION, Futtsu-shi, Chiba 293-8511 (JP); YAMAMOTO, Takeshi, NIPPON STEEL CORP. SAKAI WORKS, Sakai-shi, Osaka 590-0901 (JP); SAIKI, Eiji, NIPPON STEEL CORP. KIMITSU WORKS, Kimitsu-shi, Chiba 299-1193 (JP); KUROKAWA, Masao, NIPPON STEEL CORP. SAKAI WORKS, Sakai-shi, Osaka 590-0901 (JP)
(74) Representative: Vossius & Partner
(86) International application number: PCT/JP2001/002931
(87) International publication number: WO 2001/075182

(56) References cited:
- EP-A- 0 589 424
- EP-A- 0 940 477
- EP-A2- 0 609 556
- JP-A- 9 137 218
- JP-A- 53 057 116
- US-A- 5 738 739

## Description

The present invention relates to a method of producing an H-section used as a member for building structures and, in particular, to a rolled H-section having uniform microstructures and uniform mechanical properties.

The cross-sectional dimensions of section steels, for example H-sections, produced by hot rolling greatly vary depending on the sizes of products, and there may be cases where the amounts of rolling reduction at the time of rolling and temperature histories during and after the rolling greatly vary depending on positions in a cross section. With respect to an H-section in particular, a 1/2 flange portion (hereinafter referred to as a fillet portion) within a flange portion, at which the flange and a web are joined together, is **characterized in that** the amount of strain caused by rolling is small as compared with the other portions of the flange and, in addition to that, this portion is forcedly worked in a high temperature range. As a result of this, within the very same member, microstructural disparities are generated among different positions in a cross section of a flange portion thereof. These microstructural disparities have an influence on mechanical properties such as strength and toughness and, more specifically, constitute a main factor in decreasing the strength and toughness of a fillet portion. Such disparities in material quality within a cross section tend to stand out in the case of a large size and a thick wall size, and tend to stand out in the case of a heavy building structure using such H-sections.

To cope with the problems mentioned above, the prescribed values of mechanical properties such as strength and toughness have so far been assured by making up for decreases in the strength and toughness of a fillet portion, that is the weakest portion, by a method of increasing the addition amount of alloy or the like. In such a case, the mechanical properties of portions other than a fillet portion are superior to those of the fillet portion and are distributed at a level sufficient to satisfy the prescribed values; however, there is a case where a member having disparities in material quality within a cross section of a flange portion is inappropriate for use in a stricter steel structure design. That is to say, a problem arising in a case where an accidental large load is imposed on such a member is that cracks originate in a fillet portion. When a conventional H-section is used as a member of a structure designed to be earthquake-proof, for example, there is a danger that, when a large earthquake happens, a collapse pattern unpredictable at a designing stage may occur due to disparities in material quality generated within a cross section of the member.

In the meantime, to employ production conditions, such as alloys, processes and the like, for assuring the mechanical properties of a fillet portion, namely the weakest portion, results in the excessive assurance of the mechanical properties of the other cross-sectional positions in excess of their prescribed lower limits. Then, the excessive assurance produces the problems of inefficiency and lack of economy entailing an unnecessary price increase of a steel material. Besides, another problem here is that a flange portion and a web portion are different from each other in their microstructures because there are differences between the two in their reduction ratios and rolling temperature histories. Accordingly, it is essential to decrease the disparities in material quality within a cross section in order to more economically produce H-sections of the same specifications.

As a technology of producing an H-section having more uniform mechanical properties in view of the above described problems, envisaged is a production method of combining controlled rolling with accelerated cooling by cooling the outside surface of a flange with water, as disclosed in Japanese Unexamined Patent Publication No. H6-228634 for example. By this technology, it is possible to bring the rolling temperature history of a 1/4 flange and that of a fillet close to each other and to uniformalize the mechanical properties in a cross section of the flange portion by adjusting the water distribution in the width direction on the outside surface of the flange, namely, by convergently cooling with water the vicinity of the center of the flange width, which corresponds to the fillet, but it is difficult to uniformalize the microstructures and to sufficiently suppress disparities in strength by controlling the temperature distribution over the entire cross section including a web before the start of the water cooling and during the water cooling only using water cooling.

Further, envisaged is a method of controlling microstructures by making use of the introduction of working strain caused by a large-reduction rolling in a rolling stage and subsequent recuperation and recrystallization phenomena. However, in the case of rolling H-sections, it has so far been impossible to uniformalize the microstructures because of the restrictions on their production as it is shown hereafter.

The production processes of an H-section consists of a breakdown process for rolling a heated cast steel into an H-shaped rough form (hereinafter referred to as a rough formed cast steel) and intermediate and finish rolling processes for forming it into a product having prescribed sizes in thickness, width and height. According to a conventional production method, a cast steel is formed so that the proportion of the flange thickness of a rough formed cast steel finished in a breakdown process to the web thickness thereof comes close to the proportion of the flange thickness of a product to the web thickness thereof. This is required in order to prevent shape defects of a steel product in the longitudinal direction, such as web waves (caused by web buckling) and flange tears (caused by a difference in elongation between end portions), and defects thereof in dimensions such as thickness, width and height; these defects are developed when the proportion of the reduction of a flange thickness to that of a web thickness considerably deviates from 1 in subsequent intermediate and finish rolling processes, in particular, in a flange-web simultaneous reduction process called universal rolling.

Since the thickness of a web is thinner than that of a flange in the size of an H-section, in most cases, the above-mentioned rolling method tends to cause the temperature of a web to drop remarkably during rolling and to increase the temperature variations within an H-shaped cross section. In such a case, the distribution of temperatures shows the maximum value at a fillet and the minimum value at the middle of a web, and the temperature difference between them becomes as large as 150 to 200C in some cases.

When controlled rolling is carried out by utilizing recuperation and recrystallization with the aim of uniformly fining microstructures while temperature variations exist within an H-shaped cross section, it is necessary to apply a large-reduction rolling to each of a flange, a fillet and a web at each appropriate time, respectively. If a rolling is carried out with the proportion of the reduction of a flange thickness to that of a web thickness being close to 1 as mentioned above, a large-reduction rolling must be applied in a wide temperature range.

In order to achieve this, it is essential to increase the cross-sectional size of a rough formed cast steel finished in a breakdown process, and this in turn requires the size increase of a cast steel that is a raw material and a new formative technology of producing a rough formed cast steel having a large cross section in the breakdown process. These have been difficult to achieve as they have involved economical problems caused by a decrease in casting work efficiency and the like and technical problems such as the development of a yet-to-be achieved production method of a rough formed cast steel having a large cross section.

Accordingly, in an existing process, universal rolling has been carried out by controlling each of the reduction ratios of a flange and a web to at most 15 to 18% per pass in the temperature range from 950 to 1,100C.

As a method of fining microstructures, which is substituted for a method of rolling and water cooling control, there is a production method wherein microstructures are fined and uniformalized, even under the condition of a low reduction ratio, by dispersing intragranular ferrite transformation nuclei in austenite, as disclosed in Japanese Unexamined Patent Publication Nos. H4-279247 and H4-279248. However, this requires controlling the amount of dissolved oxygen and the generation and dispersion of oxides serving as the intragranular ferrite transformation nuclei at the stage of steelmaking, and thus, this brings about cost increasing factors such as the augmentation of secondary refining process capability to cope with a mass production. Accordingly, this production method does not suit the production of general-purpose steels premised by mass production.

Further, as technologies for producing a large-sized or thick-wall-sized H-section in view of the above mentioned problems, proposed are the technologies of reducing the grain sizes of microstructures by utilizing the precipitation of V and N, for example, in Japanese Examined Patent Publication Nos. S62-50548 and S62-54862 and Japanese Unexamined Patent Publication No. H10-60576. However, in a case where an H-section is produced by using these technologies, though disparities in microstructures within a cross section of the H-section can be mitigated to some extent, these measures are insufficient to provide uniform microstructures and/or mechanical properties. Moreover, under the present situation, there is a problem also from the viewpoint of economical efficiency since there is a concern about an increase in the production cost caused by the addition of V.

Further, there is a so-called welded H-section produced by welding steel plates together in order to solve the above-mentioned problems. However, since it involves many production processes compared with a rolled H-section, and in addition to this, the production efficiency is low, it has problems with the economical efficiency in the H-section market and the supply capability to the market. Further, uniform microstructures and/or mechanical properties within a cross section of an H-section can not always be obtained since there are cases where the mechanical properties of a weld part differ from those of a base metal depending on weld conditions.

EP-A-0 609 559 discloses a method for producing low Ceq rolled steel shapes by controlled rolling for providing steel sections of various contours and dimensions from minimized varieties of steel compositions, where the production process comprising the steps of; intermediate hot rolling comprises water-cooling the flange portion of the rough-rolled steel section between rolling passes in the intermediate rolling to cool the surface layer of the flange to a temperature not higher than 750C, and rolling the flange portion during recuperation of the surface layer of the flange at least one time between the rolling passes with a total draft not less than 20% and at an average rolling temperature not higher than 950C, and cooling the outer surface of the flange after finishing hot rolling with a cooling rate range of 0.5-10C/sec depending on the thickness of the flange.

JP-A-9-137218 discloses a manufacture of wide flange shape for building construction excellent in refractoriness and weldability, where the steel contains C: 0.001-0.030%, Si: 0.60% or less, Mn: 0.20-3.00%, Al: 0.100% or less, Ti: 0.005-0.20%, B: 0.0003-0.0050%, N: 0.0100% or less, and further contains one or more of Mo: 0.05-0.6%, Cu: 0.7-2.0% and Ni: 0.7-2.0% and the balance being Fe and unavoidable impurities, and that the steel is produced by the steps of; reheating the steel to 1200-1350C, finishing hot rolling with a temperature difference between a web part and flange part when it becomes less than 100C and both parts of web and flange reach a temperature of more than 700C, and cooling it in air for reducing a quality fracture in the cross-sectional area of the rolled H-shape steel.

The present invention solves the above-mentioned various problems and provides a method of producing rolled H-sections of various sizes produced by hot rolling and, in particular, rolled H-sections each having uniform mechanical properties within a cross section thereof by reducing microstructural variations in respective portions of each of the H-sections of large sizes and thick-walled sizes.

This object can be achieved by the features specified in the claims.

The invention is described in detail in conjunction with the drawings, in which;

Fig. 1 is a schematic view showing the portions of an H-section and the positions where test pieces are cut out and

Fig. 2 is a graph showing the transition of the average grain size of austenite after recrystallization depending on the rolling temperature history.

As mentioned above, in a flange portion of an H-section, a 1/2 flange portion (fillet portion) at which the flange and a web are joined together has a small amount of strain caused by rolling as compared with the other portions of the flange, and in addition to that, this portion is forcedly worked in a high temperature range. Therefore, within the very same member, microstructural disparities are generated among different positions in a cross section of the flange portion and the microstructural disparities cause the strength and toughness of the fillet portion to decrease. That is, when an H-section having a web portion whose wall thickness is thinner than that of a flange portion is produced in a conventional hot rolling process, the microstructure of the web portion tends to become finer than that of the flange portion because the web portion undergoes the production conditions of comparatively low temperature and large reduction. Further, along with this, the web portion tends to have lower hardenability and a lower pearlite rate than the flange portion.

The microstructural disparities have a significant influence on strength and toughness, and more specifically, cause the yield ratio of a web portion to increase. Further, the microstructural disparities and material quality disparities tend to be conspicuous when the proportion of the thickness of a flange to that of a web is large and the thickness of the web portion is thin. In order to mitigate the low-temperature and large-reduction conditions at a web portion and to bring the rolling temperature history of the web portion close to that of a flange portion, a method of shortening the time required up to the production by rolling, more specifically, a method of limiting the extension length of a steel material, namely reducing the weight of a cast steel, and accelerating the rolling and conveying speed, has so far been tried. As a consequence, however, a measure sufficient to obtain a uniform microstructure at the respective portions in a cross section has not been taken. As mentioned above, an H-section produced by conventional production processes has material quality disparities existing between a web and a flange, and there may be a case where such an H-section is inappropriate for a member used in a strict steel structure design, depending on the conditions. For example, when a conventional H-section is used as a member of a structure designed to be earthquake-proof, there is a danger that, when a large earthquake happens, a collapse pattern unpredictable in a designing stage may occur due to the disparities in material quality generated within a cross section of the member.

Therefore, the present inventors made various studies to eliminate the above-mentioned microstructural disparities and, as a result, discovered that to control the average grain sizes of ferrite or the average rates of pearlite in microstructures on the basis of a 1/4 flange portion in a cross section of an H-section and/or to control mechanical properties such as yield strength and tensile strength at a 1/2 flange portion, a web portion and a fillet portion are important factors. This will be now explained in detail.

The mechanical properties of a steel material having microstructures mainly composed of a ferrite phase and a pearlite phase can be predicted from the grain size of ferrite and the rate of pearlite. When a deformation is imposed on this steel material, plastic deformation starts to appear in the ferrite phase which is softer than the pearlite phase, and thereby the steel material yields. In a polycrystalline structure which is seen in a regular steel material, it is generally known that the mechanical properties depend on the crystal grain size of ferrite. That is to say, it has been shown theoretically and experimentally that yield strength has dependence on the grain size of ferrite, and specifically has a linear correlation with the square root of the ferrite grain size. In the case of steel materials having the same composition in particular, the square root of the ferrite grain size and the yield strength are linked to each other by a single rectilinear relation. This shows that, if the average grain sizes of ferrite in the microstructures of the steel materials having the same composition are substantially uniformalized, the yield strengths of the steel materials become substantially equal.

In the meantime, tensile strength depends not only on the strength of ferrite which is a soft phase but also on the strength of pearlite which is a hard phase. This is because a rupture limit in a tensile test, which represents tensile strength, results from the plastic deformation of both ferrite and pearlite. Since the tensile strength of a composite structure is generally considered to be the weighted average of the tensile strengths of phases constituting the structure, the total sum of each product of the strength and the rate of a constituent phase in the structure can be used as a predictive expression of the tensile strength. In the case of a steel material mainly composed of a ferrite phase and a pearlite phase, a value acquired by adding the product of the strength and the rate of the pearlite phase to the product of the strength and the rate of the ferrite phase linearly correlates with tensile strength.

In this event, tensile strength is a quantity which depends on the grain size of ferrite and the rate of pearlite because of the two reasons that the ferrite rate is equal to a value acquired by subtracting the pearlite rate from 1 because the number of main constituent phases is two and that the dependency of tensile strength on the grain size of pearlite is negligible because the plastic deformation of pearlite is very small compared with the plastic deformation of ferrite. For example, the tensile strength of a steel material is expressed by the following experimental formula (1) according to Pickering and the strength level of a rolled steel is substantially determined by the values of alloy-designed chemical constituents, the rate of pearlite, and the grain size of ferrite: $Tensilestrength \left(MPa\right) = 15.4 ⁢ \left(19.1+1.8\left[Mn\right]+5.4\left[Si\right]+0.25\left[%pearlite\right]+0.5⁢{d}^{- 1 / 2}\right)$ where, d is a ferrite grain size (mm).

This shows that tensile strengths are substantially the same if the average grain size of ferrite and the average rate of pearlite are substantially uniform in the microstructures of steel materials having the same composition. Accordingly, in order to keep a uniform strength in a cross section of an H-section, it is indispensable to apply the process control of rolling and cooling to each portion of the cross section.

The crystal grain size of ferrite is determined by the number of ferrite transformation sites and the growth rate of the ferrite crystals during the transformation of austenite into ferrite, and depends chiefly on the following conditions: 1) the grain size of austenite just before it is transformed into ferrite, and 2) a temperature at working, the amount of strain, a cooling rate in a transformation range and the like, in a working and heat treatment represented by an accelerated cooling type controlled rolling (TMCP). Further, the rate of pearlite is mainly determined by the transformation temperature of the pearlite.

On the basis of the above-mentioned principles, the present invention actualizes the uniformity of microstructures and that of mechanical properties in a cross section of an H-section by reducing microstructural disparities among a web, a flange and a fillet of the rolled H-section formed by rolling using the methods shown hereafter. The following measures can be enumerated as methods of eliminating microstructural disparities among a 1/4 flange portion, a 1/2 flange portion and a fillet portion and uniformalizing their mechanical properties:
① To sufficiently fine the structure of austenite after recrystallization at not only a 1/4 flange portion but also a 1/2 flange portion and a fillet portion by applying a large-reduction rolling with a reduction ratio of 20% or more for example, and thereby to fine microstructures finally.
② To sufficiently fine the structure of austenite after recrystallization at not only a 1/4 flange portion but also a 1/2 flange portion and a fillet portion by rolling a material in a relatively low temperature range within a recrystallization temperature range (950C or higher, for example), and thereby to fine microstructures finally. In order to realize the rolling in a relatively low temperature range, a method of cooling the flange with water between passes can be envisaged.
③ To suppress the grain growth of ferrite by accelerated cooling using water cooling after the completion of rolling, and thereby to increase the rate of pearlite in a structure.

Further, the following measures can be enumerated as methods of eliminating microstructural disparity between a 1/4 flange portion and a 1/2 web portion:
1) To eliminate a single rolling pass which uses a pass groove for a web, called a flat pass rolling, in a breakdown process, and thereby to suppress a temperature drop in the web during the rolling. Here, in order to actualize such a process, it is essential to employ a so-called universal breakdown rolling process wherein a single rolling pass for the web is used in a universal rolling process succeeding the breakdown process.
2) To shorten the time required for rolling, and thereby to suppress an increase in temperature differences among portions in a cross section of an H-section.
3) To sufficiently fine the grain sizes of austenite structures after recrystallization at not only a 1/4 flange portion but also a fillet portion by applying a large-reduction rolling, and thereby to fine the microstructures finally.
4) To fine the grain sizes of austenite structures after recrystallization at not only a 1/4 flange portion but also a fillet portion by applying rolling in a relatively low temperature range within a recrystallization temperature range (950C or higher, for example), and thereby to fine the microstructures finally. In order to actualize the rolling in the relatively low temperature range, a method of cooling a steel material with water between rolling passes can be envisaged.
5) To bring the rolling temperature histories of three portions, namely a flange, a fillet and a web, within a non-recrystallization temperature range close to each other. As concrete methods therefor, it is sufficient to control the following items:
   - To suppress differences in total reduction ratio among the portions in the non-recrystallization temperature range.
      Differences in strain introduced by rolling among the portions are reduced if a total reduction ratio of 60% or more can be secured during the reduction from a wall thickness at the upper limit of the non-recrystallization temperature range (the upper limit being of the order of 950C in terms of a temperature at the surface of a steel material, for example, in the case of a steel containing Nb among the components of the present invention) down to the wall thickness of a product.
   - To suppress differences in finishing temperatures among the portions.
      If temperatures during a finish rolling (hereinafter referred to as finishing temperatures) at the steel material surfaces of the three portions, namely a flange, a fillet and a web, are all 860C or lower, the grain sizes of microstructures are sufficiently fined. However, if they are lower than 650C, the microstructures are partly transformed into ferrite to cause work-induced ferrite to be generated during the rolling, which deteriorates mechanical properties, in particular toughness. Therefore, the lower limit of the finishing temperature is set at 650C. Further, if the differences in finishing temperatures among the three portions can be suppressed within 50C, microstructural disparities among the portions are reduced.
6) To suppress the grain growth of ferrite by accelerated cooling at a cooling rate of 0.5 to 10.0C/sec. after the completion of rolling, and thereby to increase the rate of pearlite in a structure.

According to the present invention, as mentioned above, it is necessary that the deviations of the average grain sizes of ferrite in microstructures of a 1/2 flange portion and a fillet portion from that of a 1/4 flange portion are within 15% thereof or the deviations of the average rates of pearlite in the microstructures of a 1/2 flange portion and a fillet portion from that of a 1/4 flange portion are within 8% thereof. Here, the reasons why the range of a uniform microstructure is limited to within 15% in terms of the average grain size of ferrite and within 8% in terms of the average rate of pearlite are that the results of experiments have made it clear that, as long as these limits are maintained, it is possible to control the variations of mechanical properties such as strength and toughness to within about 5%, that is, when the average grain size of ferrite and the average rate of pearlite are within the above-mentioned limits, substantially uniform mechanical properties can be obtained.

In the case of industrial production, a certain degree of tolerance is required. With respect to tensile strength and yield strength, they can be judged to be uniform if the extent of variations is such that variations in the tensile strength and yield strength are within 5% and variations in yield ratios are within 3%. For example, if any one or more of the following conditions are satisfied, mechanical properties are determined to be uniform in a cross section of an H-section. An H-section sufficiently satisfying these conditions can be obtained by employing the production method according to the present invention.

On the basis of a 1/4 flange portion:
1) A rolled H-section having uniform mechanical properties wherein the deviations of the yield strengths of a 1/2 flange portion and a fillet portion from that of the 1/4 flange portion are within 5% thereof.
2) The deviations of the yield ratios (yield strength/tensile strength) of a 1/2 flange portion and a fillet portion from that of the 1/4 flange portion are within 3% thereof.
3) The deviations of the yield strengths and tensile strengths of a 1/2 flange portion and a fillet portion from those of the 1/4 flange portion are within 5% thereof, respectively.
4) The deviations of the yield ratios (yield strength/tensile strength) and tensile strengths of a 1/2 flange portion and a fillet portion from those of the 1/4 flange portion are within 3% and 5% thereof, respectively.
5) The deviation of the yield strength of a 1/2 web portion from that of the 1/4 flange portion is within 5% thereof.
6) The deviation of the yield ratio of a 1/2 web portion from that of the 1/4 flange portion is within 3% thereof.
7) The deviations of the yield strength and tensile strength of a 1/2 web portion from those of the 1/4 flange portion are within 5% thereof, respectively.
8) The deviations of the yield ratio and tensile strength of a 1/2 web portion from those of the 1/4 flange portion are within 3% and 5% thereof, respectively.

Next, the reason why the range of the carbon equivalent in a steel of the present invention is limited to 0.15 to 0.40 mass % will be explained hereafter. The carbon equivalent in the present invention is determined by the carbon equivalent formula C_{eq} = C + Si/24 + Mn/6 + Ni/40 + Cr/5 + Mo/4 + V/14 and it ranges from 0.15 to 0.40 mass %. This composition range corresponds to the chemical compositions of a rolled steel for general structure, a rolled steel for welded structure, a rolled steel for building structure and the like defined as SN400, SS400, SM400, SN490, SM490, etc. in the JIS standards. This composition range represents the tensile strengths of 400 MPa to 610 MPa and allows achieving high toughness and high weldability. Further, when a carbon equivalent is within this range, the microstructure of a steel having such composition is mainly composed of a ferrite phase and a pearlite phase and, as mentioned above, a mechanism comes into existence wherein the microstructure has an influence on mechanical properties. In addition, the carbon equivalent formula shown in the claims is described also in the JIS standards, and it is shown there that the lower the value is, the more excellent the weldability is. Further, with respect to toughness, it is empirically known that the lower the value of the carbon equivalent formula is, the better is the value of toughness obtained.

Further, according to the present invention, Nb at 0.005 to 0.035 mass % is added to the chemical composition satisfying the above-mentioned limited range of the carbon equivalent formula in order to improve strength and toughness. It is known that the addition of Nb acts so as to suppress recrystallization of steel. For example, even in a case where Nb at 0.005 mass %, that is the minimum amount of Nb addition, is added, a non-recrystallization temperature range can be raised to a temperature range of, for example, the order of 950C, provided that the carbon equivalent is in the range according to the present invention. Further, if the concentration of added Nb exceeds 0.035 mass %, coarse Nb-based carbides disperse, which may impair the toughness and weldability of a base metal. Therefore, the upper limit of Nb is set at 0.035 mass %.

Next, the reasons why the conditions of controlled rolling and controlled cooling are limited, which are the features of the present invention, will be explained hereafter.

The reason why the reheating temperature of a cast steel is limited to within the temperature range of 1,100 to 1,300C at the time of starting the rolling of an H-section is that heating up to 1,100C or higher is required in order to make plastic deformation easy when a section steel is produced by hot rolling, and that the upper limit is set at 1,300C from the viewpoints of the capability and economical efficiency of a reheating furnace.

A heated cast steel is then rolled and formed in the processes of rough rolling, intermediate rolling and finish rolling.
As one of the features of the rolling process according to the present invention, a large-reduction rolling with a reduction ratio of 20% or more per pass in the intermediate rolling process can be mentioned. The reason why the temperature range is limited to 950 to 1,100C when a large-reduction rolling with a reduction ratio of 20% or more per pass is adopted is that the effect of recrystallization on fining the grain size in an austenite structure is maximized within this temperature range. The more the strain is imposed during rolling, the finer the grain size in the structure of austenite after recrystallization is. In the case of a rolling with a reduction ratio of less than 20% which has so far been employed, the grain sizes of the recrystallized structures of a web and a flange have been sufficiently fined; however, the grain size of the recrystallized structure of a fillet portion has not been sufficiently fined because a work-induced strain introduced into the fillet portion has been relatively small. On the other hand, by adopting a rolling with a reduction ratio of 20% or more in the above-described temperature range, the fining of the grain size of the recrystallized structure of a fillet has sufficiently progressed and it has been possible to obtain an austenite structure having grains substantially as fine as those of the web and flange portions.

Further, the higher the frequency of large-reduction rolling with a reduction ratio of 20% or more is, the more the fining of the grain size in the austenite structure advances, as shown in Fig. 2. However, as the average grain size of austenite after recrystallization converges at a value which depends on working conditions, the effect of recrystallization per pass on fining a grain size tends to decrease as the frequency of rolling increases. In this event, a part of work-induced strain is accumulated in austenite grains, acts as ferrite transformation nuclei in the austenite grains, and has the function of fining the grain size of a microstructure finally.

Further, by adding a large-reduction rolling to a production process, the number of rolling passes is reduced, the time required to roll a reheated cast steel into an H-section of a prescribed size is shortened, and temperature differences among portions in a cross section of the H-section are reduced. That is to say, temperature differences among the portions during a rolling pass are reduced and thus variations in the temperature histories of the portions are reduced.

In addition to the conditions of a large-reduction rolling, by employing the water cooling of a flange portion between rolling passes and after the completion of rolling, the uniformalizing of the microstructures of respective portions in a cross section and the uniformalizing of the mechanical properties thereof are further accelerated.

By employing the water cooling of a flange portion between rolling passes, the temperature of a fillet gradually comes closer to the temperature of a web or that of a flange, and microstructural disparities within a cross section are further reduced. Here, with respect to the water cooling of a flange between rolling passes, a method of cooling the flange so that the surface temperature of the flange portion is cooled down to 750C or lower just after the water cooling and rolling the steel material while the surface of the steel material is recuperated is effective for fining the grain size of a microstructure, and, by applying the method at least once or by repeating it a plurality of times, the effect of fining a grain size is further exhibited. In addition, this water cooling gives a temperature gradient extending from the surface layer portion of the flange to the interior, increases the permeation of working by rolling into the interior as compared with a case where water cooling is not applied, and also gives the effect of assisting the fining of the size of grains in the inner part of the wall thickness.

The number of repetition of the water cooling and the recuperation rolling depends on the thickness of a rolled material, the thickness of a flange for example, and two or more repetitions are employed when the thickness is large. Here, a reason to limit the temperature of the surface layer portion of a cooled flange to 750C or lower is that the cooling is performed not only to lower the temperature of a rolled material but also to obtain the effect of revealing the function of suppressing the quench hardening of a surface layer portion. That is to say, a rolled material is once cooled down to the austenite-ferrite transformation temperature (Ar₃ temperature) or lower by water cooling to transform austenite into ferrite, and undergoes a process of rolling the material in the austenite-ferrite two-phase domain and a process of transforming the ferrite, which is transformed once by recuperating heat and raising the temperature before the subsequent rolling pass, into austenite again as a reverse transformation, and by these processes, the grain size of the microstructure in the surface layer portion is fined, the hardenability can be remarkably lowered, and the quench-hardening of the surface layer portion can be prevented even when an accelerated cooling is applied after the completion of rolling.

Further, the purpose of finish cooling the flange portion at a cooling rate of 0.5 to 10C/sec. after the completion of rolling is to suppress the grain growth of ferrite by an accelerated cooling and thus to uniformalize the microstructures of the respective portions in the cross section with their grains being kept fine, and also to increase the rate of pearlite in a structure and thus to obtain targeted strength with the small amounts of alloys.

### Examples

The present invention will be explained hereafter based on examples.

### <Example 1>

Experimentally produced steels were melted and refined in a basic oxygen furnace and cast into cast steels 240 to 300 mm in thickness by a continuous casting method, and the cast steels were heated and then rolled into H-sections.

As the conditions for the hot rolling, employed was an H-section production method comprising a breakdown process basically by the use of groove rolling, an intermediate rolling process by the use of a group of intermediate universal mills comprising an edger mill and a universal mill, and a finish rolling process by the use of a universal mill. Here, this method may include an additional skew-roll rolling process for controlling the height of the web of an H-section.

Under this production method by rolling, in the breakdown process, a cast steel is shaped so as to have a proper flange width and web height by being rolled in the width direction of the cast steel by the use of rolling rolls each having a plurality of grooves disposed therein, each of which grooves has a projection in the center of the groove bottom which width is different from those of other grooves. In succession, in the intermediate rolling process, the flange width is shaped by the edger mill, and the web thickness and the flange thickness are shaped by the universal mill. Further, in the finish rolling process, the steel is shaped by the finishing mill into the prescribed size of an H-section.

On the other hand, in the conventional method, a cast steel undergoes the above-mentioned rolling in a breakdown process and thereafter a single web rolling process by the use of grooves, called flat pass rolling. However, the reduction of the thickness of the web in the early stage in consequence of the single web rolling causes the temperature drops of the web in the succeeding processes to be conspicuous, and the web has to be rolled in a low temperature range as compared with the other portions. Further, since a reduction ratio per pass in the universal mill is relatively small in the intermediate rolling process, the time needed for the production by rolling is prolonged, temperature differences among the portions are expanded accordingly, and that causes the disparities of rolling temperature histories.

In this example, the uniformity of microstructures and the uniformity of mechanical properties such as tensile strength and yield strength were achieved by eliminating the flat pass rolling in the breakdown process and shortening the time required for the production by rolling by using large-reduction rolling in the intermediate rolling process. For example, microstructures shown in Table 1 were obtained when the above-mentioned process was used to produce H-sections each having a web thickness of 9 mm, a flange thickness of 12 mm, a web height of 500 mm and a flange width of 200 mm, and H-sections of large size each having a web thickness of 40 mm, a flange thickness of 60 mm, a web height of 500 mm and a flange width of 500 mm. In addition, the mechanical properties of an H-section according to the present invention, which uniformalizes strength within a cross section, can be obtained not only in the cases of the above-described sizes but also similarly in the cases of, for example, an H-section of heavy wall thickness having a web thickness of 40 mm, a flange thickness of 60 mm, a web height of 500 mm and a flange width of 500 mm, and an H-section of large size having a web thickness of 19 mm, a flange thickness of 37 mm, a web height of 300 mm and a flange width of 900 mm.

The mechanical properties of the H-sections thus produced were obtained by taking test pieces from positions at 1/4 and 1/2 (1/4B and 1/2B) of the total width (B) of a flange 2 along the center line located in the center (1/2t₂) of the wall thickness t₂ of the flange 2, and from a position at 1/2 (1/2H) of the height of the web along the center line located in the center of the wall thickness of a web 3, as shown in Fig. 1. Here, 1/4B corresponds to a 1/4 flange portion, 1/2B to a fillet portion or 1/2 flange portion, and 1/2H to a 1/2 web portion. The reason why these portions are selected to evaluate the properties is that the 1/4 flange portion (1/4B) and the fillet portion (1/2B) can be considered to represent the properties of the flange portion of an H-section. Here, measurement was carried out on a cross section of an H-section in every case.

Table 1 shows the results of measuring the average grain sizes of ferrite and the average rates of pearlite in the microstructures of a 1/4 flange portion, a fillet portion and a 1/2 web portion, and proportions between those values of two portions, namely a 1/4 flange portion and a fillet portion, and between those values of two portions, namely a 1/4 flange portion and a 1/2 web portion, with respect to each of the experimentally produced steels. In the stage of production, whereas the average grain sizes of ferrite and the average rates of pearlite of the steels according to the present invention distribute in the ranges specified by the present invention, those of conventional steels (comparative steels) do not satisfy the ranges specified by the present invention and therefore desired strength or toughness has not been achieved. Here, a method of measuring the average grain sizes of ferrite and the average rates of pearlite based on microstructural observation is not specifically restricted. At least an optical microscope can be used for the observation, and when an average value is to be obtained, it is desirable to measure each value in a visual field about 0.4 mm x about 0.4 mm or larger in size within a domain in which local variations in an observed portion are judged to be sufficiently small.

**[Table 1] Flange portion microstructure measurement results of invented steels and conventional steels (comparative steels)**

| | No. | Name of portion | Position in Fig. 1 | Average ferrite grain size | Grain size proportion *1 | Average pearlite rate | Proportion of rate *1 |
|---|---|---|---|---|---|---|---|
| | | | | (m) | (%) | (%) | (%) |
| Invented steel | 1 | 1/4 flange, | 1/4B 1/2t | 16.2 | | 21.0 | |
| | | fillet, | 1/2B 1/2t | 17.8 | 9.9 | 19.1 | -9.0 |
| | | 1/2 web | 1/2W 1/2t | 12.6 | -22.2 | 23.4 | 11.4 |
| | 2 | 1/4 flange, | 1/4B 1/2t | 14.7 | | 16.7 | |
| | | fillet, | 1/2B 1/2t | 17.2 | 17.0 | 15.7 | -6.0 |
| | | 1/2 web | 1/2W 1/2t | 11.9 | -19.0 | 18.7 | 12.0 |
| | 3 | 1/4 flange, | 1/4B 1/2t | 18.2 | | 35.4 | |
| | | fillet, | 1/2B 1/2t | 21.4 | 17.6 | 31.5 | -11.0 |
| | | 1/2 web | 1/2W 1/2t | 16.1 | -11.5 | 38.7 | 9.3 |
| | 4 | 1/4 flange, | 1/4B 1/2t | 10.5 | | 19.8 | |
| | | fillet, | 1/2B 1/2t | 13.4 | 27.6 | 17.9 | -9.6 |
| | | 1/2 web | 1/2W 1/2t | 8.7 | -17.1 | 21.1 | 6.6 |
| | 5 | 1/4 flange, | 1/4B 1/2t | 9.2 | | 17.2 | |
| | | fillet, | 1/2B 1/2t | 10.3 | 12.0 | 17.1 | -0.6 |
| | | 1/2 web | 1/2W 1/2t | 7.5 | -18.5 | 19.3 | 12.2 |
| | 6 | 1/4 flange, | 1/4B 1/2t | 13.4 | | 9.8 | |
| | | fillet, | 1/2B 1/2t | 15.7 | 17.2 | 8.8 | -10.2 |
| | | 1/2 web | 1/2W 1/2t | 13.5 | 0.7 | 10.3 | 5.1 |
| | 7 | 1/4 flange, | 1/4B 1/2t | 11.2 | | 42.1 | |
| | | fillet, | 1/2B 1/2t | 11.9 | 6.3 | 41.3 | -1.9 |
| | | 1/2 web | 1/2W 1/2t | 9.9 | -11.6 | 46.1 | 9.5 |
| | 8 | 1/4 flange, | 1/4B 1/2t | 17.8 | | 39.6 | |
| | | fillet, | 1/2B 1/2t | 20.1 | 12.9 | 35.7 | -9.8 |
| | | 1/2 web | 1/2W 1/2t | 17.1 | -3.9 | 41.0 | 3.5 |
| | 9 | 1/4 flange, | 1/4B 1/2t | 8.1 | | 18.2 | |
| | | fillet, | 1/2B 1/2t | 9.1 | 12.3 | 16.9 | -7.1 |
| | | 1/2 web | 1/2W 1/2t | 6.7 | -17.3 | 19.6 | 7.7 |
| | 10 | 1/4 flange, | 1/4B 1/2t | 10.8 | | 6.1 | |
| | | fillet, | 1/2B 1/2t | 12.8 | 18.5 | 5.8 | -4.9 |
| | | 1/2 web | 1/2W 1/2t | 9.7 | -10.2 | 6.5 | 6.6 |
| | 11 | 1/4 flange, | 1/4B 1/2t | 8.1 | | 17.2 | |
| | | fillet, | 1/2B 1/2t | 8.7 | 7.4 | 16.2 | -5.8 |
| | | 1/2 web | 1/2W 1/2t | 8.2 | 1.2 | 16.6 | -3.5 |
| | 12 | 1/4 flange, | 1/4B 1/2t | 14.2 | | 16.2 | |
| | | fillet, | 1/28 1/2t | 16.0 | 12.7 | 15.1 | -6.8 |
| | | 1/2 web | 1/2W 1/2t | 12.5 | -12.0 | 16.8 | 3.7 |
| Comparative steel | 13 | 1/4 flange, | 1/4B 1/2t | 10.1 | | 16.7 | |
| | | fillet, | 1/2B 1/2t | 12.2 | 20.8 | 14.3 | -14.1 |
| | | 1/2 web | 1/2W 1/2t | 8.3 | -17.8 | 18.5 | 11.1 |
| | 14 | 1/4 flange, | 1/4B 1/2t | 9.2 | | 16.2 | |
| | | fillet, | 1/2B 1/2t | 12.4 | 34.8 | 14.5 | -10.7 |
| | | 1/2 web | 1/2W 1/2t | 7.4 | -19.6 | 19.4 | 19.5 |
| | 15 | 1/4 flange, | 1/4B 1/2t | 8.6 | | 14.5 | |
| | | fillet, | 1/2B 1/2t | 12.2 | 41.9 | 12.3 | -15.2 |
| | | 1/2 web | 1/2W 1/2t | 6.6 | -23.3 | 16.5 | 13.8 |
| | 16 | 1/4 flange, | 1/4B 1/2t | 21.5 | | 42.7 | |
| | | fillet, | 1/2B 1/2t | 25.4 | 18.1 | 38.7 | -9.4 |
| | | 1/2 web | 1/2W 1/2t | 16.4 | -23.7 | 48.1 | 12.6 |
| | 17 | 1/4 flange, | 1/4B 1/2t | 18.1 | | 39.5 | |
| | | fillet, | 1/2B 1/2t | 22.1 | 22.1 | 35.8 | -9.4 |
| | | 1/2 web | 1/2W 1/2t | 13.2 | -27.1 | 43.4 | 9.9 |
| | 18 | 1/4 flange, | 1/4B 1/2t | 12.1 | | 20.1 | |
| | | fillet, | 1/2B 1/2t | 14.8 | 22.3 | 18.1 | -10.0 |
| | | 1/2 web | 1/2W 1/2t | 9.8 | -19.0 | 22.4 | 11.4 |
| | 19 | 1/4 flange, | 1/4B 1/2t | 8.9 | | 22.8 | |
| | | fillet, | 1/2B 1/2t | 10.5 | 18.0 | 20.6 | -9.6 |
| | | 1/2 web | 1/2W 1/2t | 7.1 | -20.2 | 25.1 | 10.1 |
| | 20 | 1/4 flange, | 1/4B 1/2t | 12.3 | | 23.6 | |
| | | fillet, | 1/2B 1/2t | 15.1 | 22.8 | 20.4 | -13.6 |
| | | 1/2 web | 1/2W 1/2t | 9.9 | -19.5 | 26.5 | 12.3 |

| | | | | | | | |
|---|---|---|---|---|---|---|---|
| *1: ((fillet portion/1/4 flange portion) - 1)*100 (%) or ((1/2 web portion/1/4 flange portion) - 1)*100 (%) | | | | | | | |

### <Example 2>

It has been made clear that an H-section having uniform microstructures at three portions, namely a 1/4 flange portion, a fillet portion and a 1/2 web portion, can be produced by setting the reduction ratio of a large-reduction rolling at 20% or more in an intermediate rolling process and further combining appropriately the following rolling temperature conditions with the cooling conditions between rolling passes and after rolling as shown in Table 2, under the rolling method described in Example 1.
- Variations in the finish rolling temperatures are within 50C among three portions, namely a 1/4 flange portion, a fillet portion and a 1/2 web portion.
- Finish rolling temperatures are not lower than 650C and not higher than 860C at the three portions, namely a 1/4 flange portion, a fillet portion and a 1/2 web portion.
- A total reduction ratio in the temperature range of 950C or lower is 60% or more at both a flange portion and a web portion (here, this condition is restricted only to a case where Nb is added).
- The surface layer portion of a flange is cooled down to 750C or lower by cooling the flange with water between passes and the material is rolled during the recuperation between passes.
- The average cooling rate of an accelerated cooling with water is 0.5 to 10C/sec. after the completion of rolling until the temperature reaches 500C.

In addition, the combination of the production conditions of the invented steels in Table 1 is shown in Table 2.

**Table 2**

| Major division | No. | Name of portion | Position in Fig. 1 | Frequency of large-reduction passes (time) *1 | Fre-quency of passes with water cooling (time) *2 | Finish rolling temperature | Maximum difference in finishing temperature | Total reduction ratio in the temperature range of 950 or lower | Cooling rate after rolling | Carbon equivalent, | Nb concentration | Average ferrite grain size | *5 Maximum deviation | Pearlite rate | *5 Maximum deviation |
|---|---|---|---|---|---|---|---|---|---|---|---|---|---|---|---|
| | | | | | | | | | (C/s)*3 | (%) *4 | | | | | |
| | 1 | 1/4 flange, | 1/4F | Flange: 0 | 0 | 879 | 37 | (Less than 60%) | (Natural cooling) | 0.36 | 0.000% | 10.5 | 12.4% | 18.8% | 1.6% |
| | | fillet, | 1/2F | | | 900 | | (Less than 60%) | | | | 11.8 | -2.9% | 17.6% | -6.4% |
| | | 1/2 web | 1/2W | web: 0 | | 863 | | (Less than 60%) | | | | 10.2 | | 19.1% | |
| | 2 | 1/4 flange, | 1/4F | Flange: 3 | 0 | 910 | 31 | (Less than 60%) | (Natural cooling) | 0.30 | 0.000% | 11.8 | 4.2% | 14.8% | 2.0% |
| | | fillet, | 1/2F | | | 922 | | (Less than 60%) | | | | 12.3 | -5.1% | 15.1% | -3.4% |
| | | 1/2 web | 1/2W | Web: 3 | | 891 | | (Less than 60%) | | | | 11.2 | | 14.3% | |
| | 3 | 1/4 flange, | 1/4F | Flange: 3 | 0 | 886 | 25 | 84.6 | (Natural cooling) | 0.36 | 0.014% | 6.3 | 8.6% | 20.1% | 5.0% |
| | | fillet, | 1/2F | | | 911 | | 62.6 | | | | 6.8 | -1.4% | 21.1% | -0.0% |
| | | 1/2 web | 1/2W | Web: 3 | | 889 | | 68.5 | | | | 6.2 | | 20.5% | |
| | 4 | 1/4 flange, | 1/4F | Flange: 3 | 0 | 845 | 20 | 80.0 | (Natural cooling) | 0.38 | 0.010% | 8.7 | 11.5% | 19.6% | 1.5% |
| | | fillet, | 1/2F | | | 853 | | 59.8 | | | | 9.7 | -10.3% | 19.9% | -2.0% |
| | | 1/2 web | 1/2W | Web: 4 | | 833 | | 66.1 | | | | 7.8 | | 19.2% | |
| | 5 | 1/4 flange, | 1/4F | Flange: 2 | 0 | 799 | 22 | 76.0 | (Natural cooling) | 0.38 | 0.009% | 6.4 | 3.1% | 19.9% | 1.0% |
| | | fillet, | 1/2F | | | 812 | | 63.4 | | | | 6.6 | -1.6% | 19.5% | -2.0% |
| | | 1/2 web | 1/2W | Web: 2 | | 790 | | 70.4 | | | | 6.3 | | 20.1% | |
| | 6 | 1/4 flange, | 1/4F | Flange: 2 | 2 | 884 | 17 | (Less than 60%) | (Natural cooling) | 0.29 | 0.000% | 8.8 | 11.4% | 15.1% | 1.3% |
| | | fillet, | 1/2F | | | 901 | | (Less than 60%) | | | | 9.8 | -0.0% | 15.3% | -3.3% |
| | | 1/2 web | 1/2W | Web: 3 | | 887 | | (Less than 60%) | | | | 8.8 | | 14.6% | |
| | 7 | 1/4 flange, | 1/4F | Flange: 3 | 2 | 862 | 28 | 84.6 | (Natural cooling) | 0.38 | 0.014% | 6.5 | 0.0% | 20.0% | 4.5% |
| | | fillet, | 1/2F | | | 887 | | 62.6 | | | | 6.5 | -3.1% | 20.9% | -1.0% |
| | | 1/2 web | 1/2W | Web: 3 | | 859 | | 68.5 | | | | 6.3 | | 19.8% | |
| | 8 | 1/4 flange, | 1/4F | Flange: 3 | 0 | 834 | 35 | (Less than 60%) | (Natural cooling) | 0.29 | 0.000% | 8.3 | 9.6% | 15.1% | 2.6% |
| | | fillet, | 1/2F | | | 852 | | (Less than 60%) | | | | 9.1 | -4.8% | 15.5% | -1.3% |
| | | 1/2 web | 1/2W ' | Web: 3 | | 817 | | (Less than 60%) | | | | 7.9 | | 14.9% | |
| | 9 | 1/4 flange, | 1/4F | Flange: 1 | 4 | 807 | 27 | (Less than 60%) | (Natural cooling) | 0.32 | 0.000% | 8.6 | 3.5% | 15.2% | 1.3% |
| | | fillet, | 1/2F | | | 620 | | (Less than 60%). | | | | 8.9 | -5.8% | 15.4% | -1.3% |
| | | 1/2 web | 1/2W | Web: 1 | | 793 | | (Less than 60%) | | | | 8.1 | | 15.0% | |
| | 10 | 1/4 flange, | 1/4F | Flange: 3 | 4 | 796 | 33 | 80.0 | (Natural cooling) | 0.36 | 0.010% | 6.3 | 8.6% | 18.6% | 1.1% |
| | | fillet, | 1/2F | | | 807 | | 61.0 | | | | 6.8 | -1.4% | 18.8% | -3.8% |
| | | 1/2 web | 1/2W | Web: 4 | | 774 | | 66.1 | | | | 6.2 | | 17.9% | |
| | 11 | 1/4 flange, | 1/4F | Flange: 3 | 0 | 901 | 36 | (Less than 60%) | 1.8 | 0.36 | 0.000% | 10.1 | 6.9% | 16.1% | 6.8% |
| | | fillet, | 1/2F | | | 934 | | (Less than 60%) | 1.6 | | | 10.8 | -4.0% | 17.2% | -1.9% |
| | | 1/2 web | 1/2W | Web: 3 | | 898 | | (Less than 60%) | 1.8 | | | 9.7 | | 15.8% | |
| | 12 | 1/4 flange, | 1/4F | Flange: 3 | 0 | 887 | 33 | 84.6 | 0.9 | 0.38 | 0.011% | 9.9 | 9,1% | 18.4% | 6.0% |
| | | fillet, | 1/2F | | | 902 | | 62.6 | 0.8 | | | 10.8 | -1.0% | 19.5% | -4.9% |
| | | 1/2 web | 1/2W | Web: 3 | | 869 | | 68.5 | 0.9 | | | 9.8 | | 17.5% | |
| | 13 | 1/4 flange, | 1/4F | Flange: 3 | 0 | 842 | 24 | (Less than 60%) | 1.8 | 0.28 | 0.000% | 8.9 | 3.4% | 15.1% | 2.6% |
| | | fillet, | 1/2F | | | 855 | | (Less than 60%) | 1.6 | | | 9.2 | -2.2% | 15.5% | -5.3% |
| | | 1/2 web | 1/2W | Web: 3 | | 831 | | (Less than 60%) | 1.8 | | | 8.7 | | 14.3% | |
| | 14 | 1/4 flange, | 1/4F | Flange: 3 | 0 | 831 | 11 | 80.0 | 1.5 | 0.36 | 0.010% | 6.3 | 8.6% | 19.0% | 1.6% |
| | | fillet, | 1/2F | | | 842 | | 61.0 | 1.2 | | | 6.8 | -1.4% | 19.3% | -3.7% |
| Invented steel | | 1/2 web | 1/2W | web: 4 | | 841 | | 66.1 | 1.6 | | | 6.2 | | 18.3% | |
| | 15 | 1/4 flange, | 1/4F | Flange: 2 | 2 | 863 | 38 | (Less than 60%) | 1.6 | 0.29 | 0.000% | 8.2 | 4.9% | 15.3% | 5.9% |
| | | fillet, | 1/2F | | | 872 | | (Less than 60%) | 1.4 | | | 8.6 | -3.7% | 16.2% | -5.2% |
| | | 1/2 web | 1/2W | Web: 2 | | 834 | | (Less than 60%) | 1.7 | | | 7.9 | | 14.5% | |
| | 16 | 1/4 flange, | 1/4F | Flange: 2 | 1 | 877 | 24 | 84.6 | 1.4 | 0.38 | 0.014% | 9.1 | 3.3% | 17.8% | 6.7% |
| | | fillet, | 1/2F | | | 889 | | 62.6 | 1.3 | | | 9.4 | -3.3% | 19.0% | -7.9% |
| | | 1/2 web | 1/2W | Web: 3 | | 865 | | 68.5 | 1.6 | | | 8.8 | | 16.4% | |
| | 17 | 1/4 flange, | 1/4F | Flange: 1 | 4 | 796 | 41 | (Less than 60%) | 3.1 | 0.30 | 0.000% | 7.7 | 0.0% | 14.6% | 0.7% |
| | | fillet, | 1/2F | | | 815 | | (Less than 60%) | 2.7 | | | 7.6 | -2.6% | 14.7% | -3.4% |
| | | 1/2 web | 1/2W | Web: 1 | | 774 | | (Less than 60%) | 3.2 | | | 7.5 | | 14.1% | |
| | 18 | 1/4 flange, | 1/4F | Flange: 3 | 2 | 804 | 23 | 78.0 | 0.9 | 0.38 | 0.010% | 8.7 | 11.5% | 18.2% | 3.3% |
| | | fillet, | 1/2F | | | 820 | | (Less than 60%) | 0.8 | | | 9.7 | -10.3% | 18.8% | -1.1% |
| | | 1/2 web | 1/2W | Web: 4 | | 797 | | 64.0 | 0.9 | | | 7.8 | | 18.0% | |
| | 19 | 1/4 flange, | 1/4F | Flange: 3 | 4 | 796 | 27 | 84.6 | 3.4 | 0.36 | 0.014% | 6.3 | 8.6% | 18.5% | 0.0% |
| | | fillet, | 1/2F | | | 801 | | 62.6 | 3.2 | | | 6.8 | -1.4% | 18.5% | -2.2% |
| | | 1/2 web | 1/2W | Web: 3 | | 774 | | 68.5 | 3.6 | | | 6.2 | | 18.1% | |
| | 20 | 1/4 flange, | 1/4F | Flange:: 0 | 0 | 807 | 37 | 80.0 | (Natural cooling) | 0.34 | 0.010% | 8.7 | 11.5% | 18.9% | 5.9% |
| | | fillet, | 1/2F | | | 820 | | (Less than 60%) 66.1 | | | | 9.7 | -10.3% | 18.7% | -1.1% |
| | | 1/2 web | 1/2W | web: 0 | | 783 | | | | | | 7.8 | | 20.0% | |
| | 21 | 1/4 flange, | 1/4F | Flange: 0 | 0 | 796 | 41 | 84.6 | (Natural | 0.36 | 0.010% | 6.3 | 8.6% | 20.1% | 0.0% |
| | | fillet, | 1/2F | | | 815 | | 62.6 | cooling) | | | 6.8 | -1.4% | 18.9% | -6.0% |
| | | 1/2 web | 1/2W | Web: 0 | | 774 | | 68.5 | | | | 6.2 | | 20.0% | |
| | 22 | 1/4 flange, | 1/4F | Flange: 0 | 1 | 866 | 44 | 84.6 | (Natural | 0.35 | 0.011% | 8.4 | 8.3% | 18.1% | 7.2% |
| | | fillet, | 1/2F | | | 876 | | 62.6 | cooling) | | | 9.1 | -11.9% | 19.4% | -3.3% |
| | | 1/2 web | 1/2W | web: 0 | | 832 | | 68.5 | | | | 7.4 | | 17.5% | |
| | 23 | 1/4 flange, | 1/4F | Flange: 0 | 1 | 874 | 39 | 84.6 | (Natural | 0.35 | 0.011% | 8.4 | 9.5% | 18.4% | 4.9% |
| | | fillet, | 1/2F | | | 886 | | 62.6 | cooling) | | | 9.2 | -6.0% | 19.3% | -2.7% |
| | | 1/2 web | 1/2W | web: 0 | | 847 | | 68.5 | | | | 7.9 | | 17.9% | |
| | 24 | 1/4 flange, | 1/4F | Flange: 0 | 0 | 881 | 38 | 84.6 | 0.9 | 0.36 | 0.014% | 8.8 | 9.1% | 17.9% | 5.6% |
| | | fillet, | 1/2F | | | 895 | | 62.6 | 0.8 | | | 9.6 | -5.7 | 18.9% | -4.5% |
| | | 1/2 web | 1/2W | web: 0 | | 857 | | 68.5 | 0.9 | | | 8.3 | | 17.1% | |
| | 25 | 1/4 flange, | 1/4F | Flange: 0 | 0 | 880 | 30 | 80.0 | 1.5 | 0.36 | 0.025% | 8.5 | 0.0% | 17.6% | 5.7% |
| | | fillet, | 1/2F | | | 891 | | 61.0 | 1.3 | | | 8.2 | -7.1% | 18.6% | -3.4% |
| | | 1/2 web | 1/2W | Web: 0 | | 861 | | 66.1 | 1.7 | | | 7.9 | | 17.0% | |
| | 26 | 1/4 flange, | 1/4F | Flange: 0 | 4 | 841 | 29 | 80.0 | 1.4 | 0.32 | 0.020% | 8.4 | 1.2% | 14.1% | 7.8% |
| | | fillet, | 1/2F | | | 849 | | 61.0 | 1.3 | | | 8.5 | -11.9% | 15.2% | -2.1% |
| | | 1/2 web | 1/2W | web: 0 | | 812 | | 66.1 | 1.6 | | | 7.4 | | 13.8% | |
| | 27 | 1/4 flange, | 1/4F | Flange: 0 | 4 | 822 | 27 | 80.0 | 3.3 | 0.32 | 0.020% | 7.8 | 5.1% | 12.9% | 2.3% |
| | | fillet, | 1/2F | | | 829 | | 61.0 | 3.2 | | | 8.2 | -6.4% | 13.2% | -2.3% |
| | | 1/2 web | 1/2W | Web: 0 | | 802 | | 66.1 | 3.5 | | | 7.3 | | 12.6% | |
| | 28 | 1/4 flange, | 1/4F | Flange: 0 | 0 | 830 | 42 | (Less than 60%) | (Natural | 0.38 | 0.000% | 8.1 | 9.9% | 20.6% | 3.9% |
| | | fillet, | 1/2F | | | 854 | | (Less than 60%) | cooling) | | | 8.9 | -3.7% | 19.9% | -3.4% |
| | | 1/2 web | 1/2W | Web: 0 | | 812 | | (Less than 60%) | | | | 7.8 | | 21.4% | |
| | 29 | 1/4 flange, | 1/4F | Flange: 0 | 0 | 795 | 14 | (Less than 60%) | (Natural | 0.39 | 0.000% | 6.5 | 0.0% | 21.1% | 0.5% |
| | | fillet, | 1/2F | | | 800 | | (Less than 60%) | cooling) | | | 6.5 | -3.1% | 20.5% | -2.8% |
| | | 1/2 web | 1/2W | Web: 0 | | 786 | | (Less than 60%) | | | | 6.3 | | 21.2% | |
| | 30 | 1/4 flange, | 1/4F | Flange: 0 | 2 | 829 | 29 | (Less than 60%) | (Natural | 0.32 | 0.000% | 6.8 | 4.4% | 13.1% | 7.6% |
| | | fillet, | 1/2F | | | 838 | | (Less than 60%) | cooling) | | | 7.1 | -10.3% | 14.1% | -3.8% |
| | | 1/2 web | 1/2W | Web: 0 | | 809 | | (Less than 60%) | | | | 6.1 | | 12.6% | |
| | 31 | 1/4 flange, | 1/4F | Flange: 0 | 0 | 845 | 36 | (Less than 60%) | 5.4 | 0.33 | 0.000% | 6.1 | 9.8% | 12.8% | 0.8% |
| | | fillet, | 1/2F | | | 857 | | (Less than 60%) | 5.2 | | | 6.7 | -3.3% | 12.9% | 0.0% |
| | | 1/2 web | 1/2W | Web: 0 | | 821 | | (Less than 60%) | 5.9 | | | 5.9 | | 12.8% | |
| | 32 | 1/4 flange, | 1/4F | Flange: 0 | 2 | 826 | 28 | (Less than 60%) | 3.6 | 0.33 | 0.000% | 6.3 | 9.5% | 13.4% | 0.7% |
| | | fillet, | 1/2F | | | 837 | | (Less than 60%) | 3.4 | | | 6.9 | -4.8% | 13.5% | 0.0% |
| | | 1/2 web | 1/2W | Web: 0 | | 810 | | (Less than 60%) | 4.0 | | | 6.0 | | 13.4% | |
| | 33 | 1/4 flange, | 1/4F | Flange: 0 | 0 | 881 | 70 | (Less than 60%) | (Natural | 0.36 | 0.000% | 10.4 | 23.1% | 20.2% | 3.5% |
| | | fillet, | 1/2F | | | 902 | | (Less than 60%) | cooling) | | | 12.8 | -8.7% | 18.8% | -6.9% |
| | | 1/2 web | 1/2W | Web: 0 | | 832 | | (Less than 60%) | | | | 9.5 | | 20.9% | |
| | 34 | 1/4 flange, | 1/4F | Flange: 0 | 0 | 823 | 61 | (Less than 60%) | (Natural | 0.36 | 0.000% | 8.9 | 7.9% | 17.4% | 33.3% |
| | | fillet, | 1/2F | | | 836 | | (Less than 60%) | cooling) | | | 9.6 | -18.0% | 17.6% | -0.0% |
| | | 1/2 web | 1/2W | Web: 0 | | 775 | | (Less than 60%) | | | | 7.3 | | 23.2% | |
| | 35 | 1/4 flange, | 1/4F | Flange: 0 | 2 | 753 | 66 | (Less than 60%) | (Natural | 0.34 | 0.000% | 7.4 | 5.4% | 20.8% | 10.1% |
| | | fillet, | 1/2F | | | 786 | | (Less than 60%) | cooling) | | | 7.8 | -16.2% | 19.8% | -4.8% |
| | | 1/2 web | 1/2W | Web: 0 | | 720 | | (Less than 60%) | | | | 6.2 | | 22.9% | |
| | 36 | 1/4 flange, | 1/4F | Flange: 0 | 2 | 803 | 82 | (Less than 60%) | (Natural | 0.36 | 0.009% | 8.6 | 19.4% | 21.8% | 0.7% |
| | | fillet, | 1/2F | | | 827 | | (Less than 60%) | cooling) | | | 10.3 | -23.5% | 20.5% | -6.0% |
| | | 1/2 web | 1/2W | Web: 0 | | 745 | | (Less than 60%) | | | | 6.6 | | 22.0% | |
| | 37 | 1/4 flange, | 1/4F | Flange: 0 | 0 | 900 | 76 | (Less than 60%) | (Natural | 0.32 | 0.009% | 10.4 | 8.7% | 20.9% | 0.0% |
| | | fillet, | 1/2F | | | 948 | | (Less than 60%) | cooling) | | | 11.3 | -15.4% | 15.9% | -23.9% |
| | | 1/2 web | 1/2W | Web: 0 | | 872 | | (Less than 60%) | | | | 8.8 | | 18.0% | |
| | 38 | 1/4 flange, | 1/4F | Flange: 0 | 2 | 824 | 62 | 83.3 | (Natural | 0.32 | 0.009% | 7.3 | 34.0% | 20.0% | 0.0% |
| | | fillet, | 1/2F | | | 862 | | 66.2 | cooling) | | | 9.8 | -6.4% | 19.4% | -3.1% |
| | | 1/2 web | 1/2W | Web: 0 | | 800 | | 71.1 | | | | 6.8 | | 19.9% | |
| | 39 | 1/4 flange, | 1/4F | Flange: 0 | 0 | 756 | 63 | 80.2 | (Natural | 0.38 | 0.010% | 6.4 | 1.6% | 21.2% | 12.7% |
| | | fillet, | 1/2F | | | 794 | | 66.8 | cooling) | | | 6.5 | -18.8% | 20.9% | -1.4% |
| Comparative steel | | 1/2 web | 1/2W | Web: 0 | | 731 | | 82.5 | | | | 5.2 | | 23.9% | |
| | 40 | 1/4 flange, | 1/4F | Flange: 0 | 0 | 806 | 69 | 76.0 | (Natural | 0.39 | 0.020% | 6.3 | 0.0% | 23.5% | 2.6% |
| | | fillet, | 1/2F | | | 823 | | 63.4 | cooling) | | | 6.3 | -17.5% | 24.1% | -2.6% |
| | | 1/2 web | 1/2W | Web: 0 | | 754 | | 70.4 | | | | 5.2 | | 22.9% | |
| | 41 | 1/4 flange, | 1/4F | Flange: 1 | 2 | 881 | 70 | (Less than 60%) | (Natural | 0.31 | 0.000% | 10.4 | 23.1% | 20.2% | 3.5% |
| | | fillet, | 1/2F | | | 902 | | (Less than 60%) | cooling) | | | 12.8 | -8.7% | 18.8% | -6.9% |
| | | 1/2 web | 1/2W | Web: 1 | | 832 | | (Less than 60%) | | | | 9.5 | | 20.9% | |
| | 42 | 1/4 flange, | 1/4F | Flange: 1 | 4 | 823 | 61 | (Less than 60%) | (Natural | 0.31 | 0.000% | 8.9 | 7.9% | 17.4% | 33.3% |
| | | fillet, | 1/2F | | | 836 | | (Less than 60%) | cooling) | | | 9.6 | -18.0% | 17.6% | 0.0% |
| | | 1/2 web | 1/2W | Web: 1 | | 775 | | (Less than 60%) | | | | 7.3 | | 23.2% | |
| | 43 | 1/4 flange, | 1/4F | Flange: 2 | 4 | 753 | 66 | (Less than 60%) | (Natural | 0.30 | 0.000% | 7.4 | 5.4% | 20.8% | 10.1% |
| | | fillet, | 1/2F | | | 786 | | (Less than 60%) | cooling) | | | 7.8 | -16.2% | 19.8% | -4.8% |
| | | 1/2 web | 1/2W | Web: 1 | | 720 | | (Less than 60%) | | | | 6.2 | | 22.9% | |
| | 44 | 1/4 flange, | 1/4F | Flange: 2 | 4 | 803 | 82 | (Less than 60%) | (Natural | 0.37 | 0.009% | 8.6 | 19.4% | 21.8% | 0.7% |
| | | fillet, | 1/2F | | | 827 | | (Less than 60%) | cooling) | | | 10.3 | -23.5% | 20.5% | -6.0% |
| | | 1/2 web | 1/2W | Web: 0 | | 745 | | (Less than 60%) | | | | 6.6 | | 22.0% | |
| | 45 | 1/4 flange, | 1/4F | Flange: 1 | 2 | 900 | 76 | (Less than 60%) | (Natural | 0.37 | 0.009% | 10.4 | 8.7% | 20.9% | 0.0% |
| | | fillet, | 1/2F | | | 948 | | (Less than 60%) | cooling) | | | 11.3 | -15.4% | 15.9% | -23.9 % |
| | | 1/2 web | 1/2W | Web: 1 | | 872 | | (Less than 60%) | | | | 8.8 | | 18.0% | |
| | 46 | 1/4 flange, | 1/4F | Flange: 0 | 4 | 824 | 62 | 83.3 | (Natural | 0.37 | 0.009% | 7.3 | 34.0% | 20.0% | 0.0% |
| | | fillet, | 1/2F | | | 862 | | 66.2 | cooling) | | | 9.8 | -6.4% | 19.4% | -3.1% |
| | | 1/2 web | 1/2W | Web: 0 | | 800 | | 71.1 | | | | 6.8 | | 19.9% | |
| | 47 | 1/4 flange, | 1/4F | Flange: 2 | 4 | 756 | 63 | 80.2 | 1.3 | 0.39 | 0.010% | 6.4 | 1.6% | 21.2% | 12.7% |
| | | fillet, | 1/2F | | | 794 | | 66.8 | 1.1 | | | 6.5 | -18.8% | 20.9% | -1.4% |
| | | 1/2 web | 1/2W | Web: 1 | | 731 | | 82.5 | 1.6 | | | 5.2 | | 23.9% | |
| | 48 | 1/4 flange, | 1/4F | Flange: 1 | 4 | 805 | 63 | 76.0 | 1.4 | 0.39 | 0.013% | 7.5 | 4.0% | 23.5% | 2.6% |
| | | fillet, | 1/2F | | | 823 | | 63.4 | 1.1 | | | 7.8 | -16.0% | 24.1% | -2.6% |
| | | 1/2 web | 1/2W | Web: 0 | | 760 | | 70.4 | 1.7 | | | 6.3 | | 22.9% | |

| | | | | | | | | | | | | | | | |
|---|---|---|---|---|---|---|---|---|---|---|---|---|---|---|---|
| *1: Frequency of rolling passes with a reduction ratio of 20% or more per pass in the temperature range from 950 to 1,100C *2: Frequency of passes during the time when the surface layer portion of a flange is cooled down to 750C or lower by cooling the flange with water *3: Average cooling rate in the temperature range from 800 to 500C (recorded only when accelerated cooling with water is applied) *4: Carbon equivalent = C + Si/24 + Mn/6 + Ni/40 + Cr/5 + Mo/4 + V/14 *5: Deviation = ((fillet portion/1/4 flange portion) - 1)100 (%), or = ((fillet portion/1/2 web portion) - 1)100 (%) | | | | | | | | | | | | | | | |

### <Example 3>

The mechanical properties of H-sections produced by the method similar to that employed in Example 1 are shown in Table 3.

Table 3 shows the results of measuring the yield strength and tensile strength of a 1/4 flange portion, a fillet portion and a 1/2 web portion, and the proportions between those values of two portions, namely a 1/4 flange portion and a fillet portion, and between those values of two portions, namely a 1/4 flange portion and a 1/2 web portion, with respect to each of the experimentally produced steels. In a stage of production, whereas the average grain sizes of ferrite and the average rates of pearlite of the steels according to the present invention distribute in the ranges specified by the present invention, those of conventional steels (comparative steels) do not satisfy the ranges specified by the present invention and therefore desired strength or toughness has not been achieved. Here, although the size of test pieces for measuring tensile strength and yield strength is not specifically restricted, it is desirable to use at least JIS standards and a method compliant with JIS standards.

**[Table 3] Mechanical properties of respective portions in a cross section of each H-section of invented steels and conventional steels (comparative steels)**

| | Steel No. | Carbon equivalent | Name of portion | Position in Fig. 1 | Yield strength | Proportion | Tensile strength | Proportion | Yield ratio | Proportion |
|---|---|---|---|---|---|---|---|---|---|---|
| | | (%) *1 | | | (MPa) | (%) *2 | (MPa) | (%) *2 | (%) | (%) *2 |
| | 1 | 0.35 | 1/4 flange, | 1/4B 1/2t | 418 | | 545 | | 76.7 | |
| | | | fillet, | 1/2B 1/2t | 401 | 95.9 | 505 | 92.7 | 79.4 | 103.5 |
| | | | 1/2 web | 1/2W 1/2t | 440 | 105.3 | 551 | 101.1 | 79.9 | 104.1 |
| | 2 | 0.39 | 1/4 flange, | 1/4B 1/2t | 435 | | 557 | | 78.1 | |
| | | | fillet, | 1/2B 1/2t | 412 | 94.7 | 523 | 93.9 | 78.8 | 100.9 |
| | | | 1/2 web | 1/2W 1/2t | 465 | 106.9 | 575 | 103.2 | 80.9 | 103.6 |
| | 3 | 0.31 | 1/4 flange, | 1/4B 1/2t | 352 | | 461 | | 76.4 | |
| | | | fillet, | 1/2B 1/2t | 341 | 96.9 | 464 | 100.7 | 73.5 | 96.2 |
| | | | 1/2 web | 1/2W 1/2t | 384 | 109.1 | 486 | 105.4 | 79.0 | 103.5 |
| | 4 | 0.25 | 1/4 flange, | 1/4B 1/2t | 267 | | 340 | | 78.5 | |
| | | | fillet, | 1/2B 1/2t | 251 | 94.0 | 328 | 96.5 | 76.5 | 97.4 |
| | | | 1/2 web | 1/2W 1/2t | 284 | 106.4 | 377 | 110.9 | 75.3 | 95.9 |
| | 5 | 0.29 | 1/4 flange, | 1/4B 1/2t | 315 | | 412 | | 76.5 | |
| | | | fillet, | 1/2B 1/2t | 307 | 97.5 | 409 | 99.3 | 75.1 | 98.2 |
| | | | 1/2 web | 1/2W 1/2t | 344 | 109.2 | 434 | 105.3 | 79.3 | 103.7 |
| | 6 | 0.19 | 1/4 flange, | 1/4B 1/2t | 211 | | 281 | | 75.1 | |
| | | | fillet, | 1/2B 1/2t | 199 | 94.3 | 277 | 98.6 | 71.8 | 95.7 |
| | | | 1/2 web | 1/2W 1/2t | 219 | 103.8 | 302 | 107.5 | 72.5 | 96.6 |
| | 7 | 0.23 | 1/4 flange, | 1/4B 1/2t | 227 | | 295 | | 76.9 | |
| | | | fillet, | 1/2B 1/2t | 214 | 94.3 | 290 | 98.3 | 73.8 | 95.9 |
| | | | 1/2 web | 1/2W 1/2t | 241 | 106.2 | 315 | 106.8 | 76.5 | 99.4 |
| | 8 | 0.23 | 1/4 flange, | 1/4B 1/2t | 231 | | 297 | | 77.8 | |
| | | | fillet, | 1/2B 1/2t | 218 | 94.4 | 291 | 98.0 | 74.9 | 96.3 |
| | | | 1/2 web | 1/2W 1/2t | 242 | 104.8 | 301 | 101.3 | 80.4 | 103.4 |
| Invented steel | 9 | 0.23 | 1/4 flange, | 1/4B 1/2t | 235 | | 301 | | 78.1 | |
| | | | fillet, | 1/2B 1/2t | 222 | 94.5 | 294 | 97.7 | 75.5 | 96.7 |
| | | | 1/2 web | 1/2W 1/2t | 248 | 105.5 | 315 | 104.7 | 78.7 | 100.8 |
| | 10 | 0.31 | 1/4 flange, | 1/4B 1/2t | 322 | | 417 | | 77.2 | |
| | | | fillet, | 1/2B 1/2t | 304 | 94.4 | 408 | 97.8 | 74.5 | 96.5 |
| | | | 1/2 web | 1/2W 1/2t | 329 | 102.2 | 422 | 101.2 | 78.0 | 101.0 |
| | 11 | 0.31 | 1/4 flange, | 1/4B 1/2t | 328 | | 423 | | 77.5 | |
| | | | fillet, | 1/2B 1/2t | 307 | 93.6 | 410 | 96.9 | 74.9 | 96.6 |
| | | | 1/2 web | 1/2W 1/2t | 333 | 101.5 | 451 | 106.6 | 73.8 | 95.2 |
| | 12 | 0.24 | 1/4 flange, | 1/4B 1/2t | 271 | | 362 | | 74.9 | |
| | | | fillet, | 1/2B 1/2t | 259 | 95.6 | 360 | 99.4 | 71.9 | 96.1 |
| | | | 1/2 web | 1/2W 1/2t | 281 | 103.7 | 359 | 99.2 | 78.3 | 104.6 |
| | 13 | 0.25 | 1/4 flange, | 1/4B 1/2t | 244 | | 338 | | 72.2 | |
| | | | fillet, | 1/2B 1/2t | 230 | 94.3 | 312 | 92.3 | 73.7 | 102.1 |
| | | | 1/2 web | 1/2W 1/2t | 261 | 107.0 | 353 | 104.4 | 73.9 | 102.4 |
| | 14 | 0.29 | 1/4 flange, | 1/4B 1/2t | 311 | | 421 | | 73.9 | |
| | | | fillet, | 1/2B 1/2t | 290 | 93.2 | 402 | 95.5 | 72.1 | 97.7 |
| | | | 1/2 web | 1/2W 1/2t | 331 | 106.4 | 435 | 103.3 | 76.1 | 103.0 |
| | 15 | 0.30 | 1/4 flange, | 1/4B 1/2t | 312 | | 417 | | 74.8 | |
| | | | fillet, | 1/2B 1/2t | 299 | 95.8 | 413 | 99.0 | 72.4 | 96.8 |
| | | | 1/2 web | 1/2W 1/2t | 333 | 106.7 | 435 | 104.3 | 76.6 | 102.3 |
| | 16 | 0.29 | 1/4 flange, | 1/4B 1/2t | 320 | | 411 | | 77.9 | |
| | | | fillet, | 1/2B 1/2t | 302 | 94.4 | 404 | 98.3 | 74.8 | 97.2 |
| | | | 1/2 web | 1/2W 1/2t | 332 | 103.8 | 423 | 102.9 | 78.5 | 101.3 |
| | 17 | 0.37 | 1/4 flange, | 1/4B 1/2t | 419 | | 545 | | 76.9 | |
| | | | fillet, | 1/2B 1/2t | 399 | 95.2 | 534 | 98.0 | 74.7 | 97.2 |
| | | | 1/2 web | 1/2W 1/2t | 440 | 105.0 | 565 | 103.7 | 77.9 | 101.3 |
| | 18 | 0.39 | 1/4 flange, | 1/4B 1/2t | 435 | | 557 | | 78.1 | |
| | | | fillet, | 1/2B 1/2t | 422 | 97.0 | 552 | 99.1 | 76.4 | 97.9 |
| | | | 1/2 web | 1/2W 1/2t | 456 | 104.8 | 575 | 103.2 | 79.3 | 101.5 |
| | 19 | 0.39 | 1/4 flange, | 1/4B 1/2t | 430 | | 557 | | 77.2 | |
| | | | fillet, | 1/2B 1/2t | 399 | 92.8 | 545 | 97.8 | 73.2 | 94.8 |
| | | | 1/2 web | 1/2W 1/2t | 453 | 105.3 | 561 | 100.7 | 80.7 | 104.6 |
| Comparative steel | 20 | 0.39 | 1/4 flange, | 1/4B 1/2t | 431 | | 557 | | 77.4 | |
| | | | fillet, | 1/2B 1/2t | 400 | 92.8 | 546 | 98.0 | 73.3 | 94.7 |
| | | | 1/2 web | 1/2W 1/2t | 453 | 105.1 | 565 | 101.4 | 80.2 | 103.6 |
| | 21 | 0.39 | 1/4 flange, | 1/4B 1/2t | 424 | | 554 | | 76.5 | |
| | | | fillet, | 1/2B 1/2t | 386 | 91.0 | 521 | 94.0 | 74.1 | 96.8 |
| | | | 1/2 web | 1/2W 1/2t | 453 | 106.8 | 570 | 102.9 | 79.5 | 103.8 |

| | | | | | | | | | | |
|---|---|---|---|---|---|---|---|---|---|---|
| *1: Carbon equivalent = C + Si/24 + Mn/6 + Ni/40 + Cr/5 + Mo/4 + V/14 *2: ((fillet portion/1/4 flange portion) - 1)100 (%), or = ((fillet portion/1/2 web portion) - 1)100 (%) Note) Data showing the deviations of yield strength proportions and tensile strength proportions falling within 5% and the deviation of yield ratio proportions falling within 3%. | | | | | | | | | | |

As explained above, the present invention makes it possible to provide an H-section having few microstructural disparities among respective portions of the H-section and having uniform mechanical properties within a cross section of the H-section.

## Claims

1. A method of producing a rolled H-section having uniform microstructures and uniform mechanical properties, wherein the H-section is produced from a cast steel having a chemical composition containing C_{eq}, defined by the carbon equivalent formula C_{eq} = C + Si/24 + Mn/6 + Ni/40 + Cr/5 + Mo/4 + V/14, at 0.15 to 0.40 mass by rolling the cast steel one or more times with a reduction ratio of 20% or more per pass to each of a flange and a web while the average temperature along the wall thickness of a flange and a web portion is within the range between 950 and 1,100C; and the microstructures satisfy any one or more of the following conditions on the basis of a 1/4 flange portion in a cross section of said H-section by applying a finish rolling wherein the finish rolling temperatures, each expressed in terms of a surface temperature during the finish rolling, of the three portions, namely a 1/4 flange portion, a fillet portion and a 1/2 web portion in a cross section of the H-section, vary within 50C:
1) the deviations of the average grain sizes of ferrite in the microstructures of a 1/2 flange portion and a fillet portion from that of the 1/4 flange portion are within 15% thereof,
2) the deviation of the average grain size of ferrite in the microstructure of a 1/2 web portion from that of the 1/4 flange portion is within 15% thereof,
3) the deviations of the average rates of pearlite in the microstructures of a 1/2 flange portion and a fillet portion from that of the 1/4 flange portion are within 8% thereof, and
4) the deviation of the average rate of pearlite in the microstructure of a 1/2 web portion from that of the 1/4 flange portion is within 8% thereof.

2. A method of producing a rolled H-section having uniform microstructures and uniform mechanical properties according to claim 1, wherein a cast steel containing Nb of 0.005 to 0.035 mass % added further to the chemical composition according to claim 1 is finish rolled with a total reduction ratio of 60% or more at each of a flange portion and a web portion while the temperature of the surface of the steel material is 950C or lower.

3. A method of producing a rolled H-section having uniform microstructures and uniform mechanical properties according to claim 1 or 2, wherein the rolling is carried out by applying a finish rolling while each of the finish rolling temperatures of the three portions, namely a 1/4 flange portion, a fillet portion and a 1/2 web portion, is in the range from 650C to 860C.

4. A method of producing a rolled H-section having uniform microstructures and uniform mechanical properties according to claim 2 or 3, wherein the production is carried out by further applying either one of the following two processes or the combination thereof:
1) a process group wherein the process of cooling a flange to a surface layer temperature of 750C or lower by cooling the flange with water between the passes of reverse rolling in an intermediate rolling process and rolling the material during the course of heat recuperation between the passes of said reverse rolling is applied once or more times, and
2) a process of applying an accelerated cooling with water at an average cooling rate of 0.5 to 10C/sec. in the period of time after the completion of rolling in the finish rolling process until a temperature reaches 500C (here, if the process 2) is not included, natural cooling is adopted down to 500C after the completion of the rolling).

## Patentansprüche

1. Verfahren zur Herstellung eines gewalzten H-Profils mit gleichmigen Mikrostrukturen und gleichmigen mechanischen Eigenschaften, wobei das H-Profil aus einem Gustahl mit einer chemischen Zusammensetzung, die C_{eq}, definiert durch die Kohlenstffquivalentformel C_{eq} = C + Si/24 + Mn/6 + Ni/40 + Cr/5 + Mo/4 + V/14, mit 0,15 bis 0,40 Masse-% enthlt, durch ein- oder mehrmaliges Walzen des Gustahls mit einem Walzgrad von mindestens 20 % je Stich jeweils an einem Flansch und einem Steg hergestellt wird, whrend die mittlere Temperatur entlang der Wanddicke eines Flansch- und eines Stegabschnitts im Bereich zwischen 950 und 1100 C liegt; und die Mikrostrukturen mindestens eine der folgenden Bedingungen auf der Grundlage eines 1/4-Flanschabschnitts in einem Querschnitt des H-Profils durch Anwenden von Fertigwalzen erfllen, wobei die Fertigwalztemperaturen, jeweils ausgedrckt in einer Oberflchentemperatur beim Fertigwalzen, der drei Abschnitte, d. h. eines 1/4-Flanschabschnitts, eines Kehlungsabschnitts und eines 1/2-Stegabschnitts, in einem Querschnitt des H-Profils innerhalb von 50 C variieren:
1) die Abweichungen der mittleren Korngren von Ferrit in den Mikrostrukturen eines 1/2-Flanschabschnitts und eines Kehlungsabschnitts von der des 1/4-Flanschabschnitts liegen innerhalb von 15 %,
2) die Abweichung der mittleren Korngre von Ferrit in der Mikrostruktur eines 1/2-Stegabschnitts von der des 1/4-Flanschabschnitts liegt innerhalb von 15 %,
3) die Abweichungen der mittleren Raten von Perlit in den Mikrostrukturen eines 1/2-Flanschabschnitts und eines Kehlungsabschnitts von der des 1/4-Flanschabschnitts liegen innerhalb von 8 % und
4) die Abweichung der mittleren Rate von Perlit in der Mikrostruktur eines 1/2-Stegabschnitts von der des 1/4-Flanschabschnitts liegt innerhalb von 8 %.

2. Verfahren zur Herstellung eines gewalzten H-Profils mit gleichmigen Mikrostrukturen und gleichmigen mechanischen Eigenschaften nach Anspruch 1, wobei ein Gustahl, der Nb mit 0,005 bis 0,035 Masse-% enthlt, das der chemischen Zusammensetzung nach Anspruch 1 ferner zugegeben ist, mit einem Gesamtwalzgrad von mindestens 60 % jeweils an einem Flanschabschnitt und einem Stegabschnitt fertiggewalzt wird, whrend die Temperatur der Oberflche des Stahlmaterials hchstens 950 C betrgt.

3. Verfahren zur Herstellung eines gewalzten H-Profils mit gleichmigen Mikrostrukturen und gleichmigen mechanischen Eigenschaften nach Anspruch 1 oder 2, wobei das Walzen durch Anwenden, von Fertigwalzen durchgefhrt wird, whrend jede der Fertigwalztemperaturen der drei Abschnitte, d. h. eines 1/4-Flanschabschnitts, eines Kehlungsabschnitts und eines 1/2-Stegabschnitts, im Bereich von 650 C bis 860 C liegt.

4. Verfahren zur Herstellung eines gewalzten H-Profils mit gleichmigen Mikrostrukturen und gleichmigen mechanischen Eigenschaften nach Anspruch 2 oder 3, wobei die Herstellung durch weiteres Anwenden eines der folgenden beiden Prozesse oder ihrer Kombination durchgefhrt wird:
1) einer Prozegruppe, wobei der Abkhlungsproze eines Flanschs auf eine Oberflchenschichttemperatur von hchstens 750 C durch Wasserkhlung des Flanschs zwischen den Stichen von Reversierwalzen in einem Zwischenwalzproze und Walzen des Materials im Verlauf von Wrmerckgewinnung zwischen den Stichen des Reversierwalzens einmal oder mehrmals angewendet wird, und
2) eines Prozesses der Anwendung einer beschleunigten Wasserkhlung mit einer mittleren Abkhlungsgeschwindigkeit von 0,5 bis 10 C/s in der Zeitspanne nach dem Walzabschlu im Fertigwalzproze, bis eine Temperatur 500 C erreicht (ist hierbei der Proze 2) nicht eingeschlossen, kommt natrliche Abkhlung auf 500 C nach dem Abschlu des Walzens zum Einsatz).

## Revendications

1. Procd pour produire une section en forme de H lamine ayant des microstructures uniformes et des proprits mcaniques uniformes, dans lequel la section en forme de H est produite partir d'un acier moul ayant une composition chimique contenant C_{eq} dfinie par la formule en quivalent carbone :
C_{eq} = C + Si/24 + Mn/6 + Ni/40 + Cr/5 + Mo/4 + V/14 de 0,15 0,40% en poids, en laminant l'acier moul une ou plusieurs fois avec un rapport de rduction de 20% ou plus par passage sur chacun parmi un rebord et une bande alors que la temprature moyenne le long de l'paisseur de paroi d'un rebord et d'une partie de bande est comprise entre 950 et 1 100 C ; et les microstructures satisfont une ou plusieurs des conditions suivantes sur la base d'un de partie de rebord dans une section transversale de ladite section en forme de H en appliquant un laminage de finition, dans lequel les tempratures de laminage de finition, chacune exprimes en termes de temprature de surface pendant le laminage de finition, des trois parties, c'est--dire de partie de rebord, une partie de cong et partie de bande dans une section transversale de la section en forme de H, varient dans une plage de 50 C ;
1) les diffrences des tailles de grain moyennes de ferrite dans les microstructures d'une partie de rebord et d'une partie de cong par rapport celles d'un de partie de rebord sont dans une plage de 15 %,
2) la diffrence de la taille de grain moyenne de ferrite dans la microstructure d'une partie de bande par rapport celle d'un de partie de rebord est dans une plage de 15 %,
3) les diffrences de taux moyens de perlite dans les microstructures d'une partie de rebord et d'une partie de cong par rapport celles d'un de partie de rebord sont dans une plage de 8 % ; et
4) la diffrence du taux moyen de perlite dans la microstructure d'une partie de bande par rapport celle d'un de partie de rebord est dans une plage de 8 %.

2. Procd pour produire une section lamine en forme de H ayant des microstructures uniformes et des proprits mcaniques uniformes selon la revendication 1, dans lequel un acier moul contenant de 0,005 0,035 % en poids de Nb ajout la composition chimique selon la revendication 1 est lamin avec un traitement de finition ayant un rapport de rduction total de 60 % ou plus au niveau de chacune parmi une partie de rebord et une partie de bande alors que la temprature de la surface de l'acier est de 950 C ou moins.

3. Procd pour produire une section lamine en forme de H ayant des microstructures uniformes et des proprits mcaniques uniformes selon la revendication 1 ou 2, dans lequel le laminage est ralis en appliquant un laminage de finition alors que chacune des tempratures de laminage de finition des trois parties, c'est--dire de partie de rebord, une partie de cong et de partie de bande, est de l'ordre d 650 C 860 C.

4. Procd pour produire une section lamine en forme de H ayant des microstructures uniformes et des proprits mcaniques uniformes selon la revendication 2 ou 3, dans lequel la production est ralise en appliquant en outre l'un des deux procds suivants ou leur combinaison :
1) un groupe de procds dans lequel le procd consistant refroidir un rebord une temprature de couche de surface de 750 C ou moins en refroidissant le rebord avec de l'eau entre les passages du laminage invers dans un procd de laminage intermdiaire et laminer le matriau pendant la rcupration de chaleur entre les passages dudit laminage invers, est appliqu une fois ou plusieurs fois, et
2) un procd consistant appliquer un refroidissement acclr avec de l'eau une vitesse de refroidissement moyenne de 0,5 10 C/s dans la priode de temps situe aprs l'achvement du laminage dans le procd de laminage de finition jusqu' ce qu'une temprature atteigne 500 C (ici, si le procd 2 n'est pas inclus, on adopte le refroidissement naturel jusqu' 500 C aprs l'achvement du laminage).
